

May 11, 1937.

B. GÁSPÁR

2,080,041

METHOD OF PRODUCING COLOR PHOTOGRAPHIC IMAGES AND CINEMATOGRAPH  
FILMS AND LIGHT SENSITIVE EMULSION THEREFOR

Filed March 21, 1935



Inventor

Bela Gaspar,

By

F. Gerald Toyer

Attorney

## UNITED STATES PATENT OFFICE

2,080,041

## METHOD OF PRODUCING COLOR-PHOTOGRAPHIC IMAGES AND CINEMATOGRAPH FILMS AND LIGHT-SENSITIVE EMULSION THEREFOR

Belá Gáspár, Brussels, Belgium

Application March 21, 1935, Serial No. 12,254  
In Germany March 29, 1934

8 Claims.

(Cl. 95—6)

This invention relates to a method of producing single-color or multi-color photographs and cinematograph films.

It is known to produce photographic images with the assistance of materials containing the dyestuff, which is necessary for the formation of the image, in the light-sensitive layer. The absorption of the colored layers is, however, obstructive for numerous purposes in the photographic art. In particular it is impossible to sensitize the layers sufficiently in respect to the spectral ranges in which the dyestuffs perform absorption.

The subject matter of the invention is a method by which there may be obtained a sufficient amount of dyestuff as required for photographic and more particularly color-photographic purposes in such a form that the presence of the dyestuff does not prevent the light from reaching the sensitized particles even in the absorption range of the dyestuff.

It has been found that dyestuffs in coarsely dispersed form (for example, in the form of intermittently distributed particles of powder) color the binding agent merely weakly or practically not at all. The layers containing dyestuff in coarsely dispersed form are highly transparent even for light which would be absorbed if the same dyestuffs were present in dissolved or finely distributed form. According to the invention, the photographic image is produced in good transmittant layers of this kind, and after exposure the emulsion layer is fastly dyed by dissolving the coarse grains of coarsely dispersed dyestuff within the layer, whereupon the layer is rendered highly absorptive. The color intensity may be predetermined exactly by the amount of coarsely dispersed dyestuff, dispersed in the emulsion during the manufacture of the material. The latent silver image may be developed before or after the transformation of the coarsely dispersed dyestuff into finely distributed dyestuff. The dyestuff is then locally destroyed proportional to the metallic silver image.

By way of explaining the invention, reference may be had to the single figure of the accompanying drawing which represents a flow diagram showing the various steps in the practice of applicant's method.

As will be understood from the following description, the sequence of the steps in my improved method may be changed provided that the unexposed material contains the coarse grained dyestuff and that the dyestuff dissolution comes after the exposure.

The dyestuff is introduced into light-sensitive

layers, or into the solutions or emulsions employed for producing the same, in coarsely dispersed form exhibiting little or no absorption. Under these conditions there will occur merely a weak coloring and a small shading effect of the particles. The dyestuff, after the exposure, is then converted at a desired point in the treatment of the image from the coarsely dispersed, non-coloring form into the color-effective form. This is performed either by means of suitable solvents or by chemical substances which cause a diffuse coloring of the layer. It is immaterial whether these agents transform the dyestuff chemically or convert it into a colloidal or highly dispersed powerfully absorbing form.

*Example.*—Spirit Fast Red B (Ullmann, Enzyklopädie der Technischen Chemie, 2nd ed. vol. 9, page 572) in powder form is admixed with gelatine. The proportion of powdered dyestuff to gelatine must be so chosen that after pouring on to a support the powdered dyestuff is distributed intermittently; i. e., that the gelatine still possesses a good transparency. The quantity of dyestuff should also not be greater than is necessary for a sufficiently good diffuse coloring of the layer. This diffuse coloring is then obtained during the later process by converting the dyestuff into the finely dispersed color-effective form, for example by bathing in a diluted alcohol solution.

The solution must have a concentration at which on the one hand the gelatine still swells, but at which on the other hand the dyestuff is dissolved. With an excess of powdered dyestuff the shading effect is too considerable, which is detrimental to the exposure of the layer.

For producing layers which contain dyestuffs in coarsely dispersed form, dyestuffs are very suitable which are insoluble or difficultly soluble in water assuming that water-soluble or saturable binding agents (for example gelatine) are employed. For binding agents which are insoluble in water dyestuffs will be employed which are insoluble or difficultly soluble in the solvents for the binding agent.

The dyestuff is either introduced into the binding agent mechanically prior to pouring, or applied to the surface of the layer either by dusting on or by pouring on to the layer in a suspension, with or without binding agents. The dyestuff may also be dissolved in a solvent, which does not cause swelling of the binding agent and upon evaporation leaves the dyestuff as a coarsely distributed sediment.

The dyestuff may be introduced into the bind-

ing agent by means of an auxiliary solvent. For example, a water-insoluble, alcohol-soluble dyestuff is dissolved in alcohol, and introduced into gelatine solution by rapid agitation. The dyestuff will be precipitated in larger or smaller size of grain dependent on the nature of the agitation and the concentration of the dyestuff solution.

In this connection it is to be observed that in 10 the gelatine solution the alcohol should not reach that concentration at which the grains of dyestuff again dissolve. Alcoholic solutions of Quinoline Yellow—spirit-soluble (Schultz Farbstofftabellen 7th ed. vol. 1, No. 917) and the tannates 15 or abietinates of basic dyestuffs, for example of Methylene Blue (Schultz, loc. cit. No. 1038), Janus Blue (Indoine Blue B, Schultz, loc. cit. No. 286), Red (Schultz, loc. cit. No. 557) or Yellow (Schultz, loc. cit. No. 292), or of Chrysoidine (Schultz, loc. 20 cit. No. 27) are suitable. These solutions are poured into water, the dyestuff salts then being precipitated in flake or granular form. The watery suspension of these particles of dyestuff is mixed with gelatine solution. The solutions may 25 also be poured directly into the gelatine. The dyestuffs may also be dissolved in water and precipitated. After the precipitation the deposit is filtered and freed from excess of precipitating agent by washing, and then mixed with a binding 30 agent with or without a light-sensitive substance. The precipitation may also be performed in the presence of the binding agent. If there is a sufficient excess of the precipitating agent, a coarsely dispersed precipitation of the dyestuff may be obtained. In this case the conditions are the same 35 as in the preparation of the emulsion, in which it is possible by varying the known factors to obtain coarse-grain or fine-grain deposits in the layer. In addition to the basic dyestuffs afore- 40 said acid and substantive dyestuffs, such as Anthosine (Schultz, loc. cit. No. 51), Metanil Yellow (Schultz, loc. cit. No. 169), Naphthylamine Black (Schultz, loc. cit. No. 229) and Diamine Pure Blue (Schultz, loc. cit. No. 510), are also suitable. 45 These are precipitated with salts of the alkaline earths, magnesium or with heavy metal salts, such as zinc or silver salts, or also with salts of organic bases, for example aniline or naphthylamine. The difficultly soluble dyestuffs may also 50 be precipitated by the addition of salt.

The precipitation may take place both in water as well as in the presence of binding agents. The size of grain will depend only on the known factors. The binding agent solution may be allowed 55 to solidify, and freed from the soluble constituents in the usual fashion by washing.

The most suitable are very difficultly soluble dyestuffs, which dissolve in water only when hot and upon cooling are completely precipitated. 60 These may be employed without precipitating agents. The dyestuff may also be allowed to form immediately in the coarse-grain form in solution or in the binding agent from the preliminary stages or components, for example from 65 vat solutions by the rapid injection of air or from leuco-ester solutions in the presence of relatively large quantities of acid and oxidizing agents, by coupling diazo compounds with azo components, if desired in the presence of precipitating agents.

The photographic layers which contain the dyestuff in coarsely dispersed and little-absorbing or coloring form within, below or above the layers are then exposed and treated in a desired 75 photographic process. At a desired point in the

treatment of the image the dyestuffs are converted into a condition in which they develop their full coloring effect, i. e., diffusely color the layer. For diffuse coloring of the layer the coarsely dispersed dyestuff located on the surface 5 of the layer or below the layer may creep into the layer and diffusely color the same.

There are various possibilities of converting the coarsely dispersed dyestuff into the powerfully absorbing, dissolved or finely distributed form. 10 This conversion may be performed for example by treatment with solvents, which cause the coarsely dispersed particles of dyestuff to be dissolved, these being finely distributed in the layer either by chemical or physical action.

For example, a tannic salt of a basic dyestuff 15 will pass into solution with acids. It is advantageous if the acid employed possesses chemically a greater affinity for the dyestuff than that used for precipitation. Numerous salts of acid dyestuffs pass into solution with diluted alkalies or also with acids. For example, the dyestuff passes from the barium salt of chrysophenine or anthosine into solution in 1% sulphuric acid. In this case barium sulphate is formed. The barium sulphate is more difficultly soluble than the dyestuff salt, i. e., barium has a greater affinity towards the sulphate-ion, and accordingly, the dyestuff is again liberated. The coarsely dispersed grains pass into solution either in the presence of the acid or upon the subsequent washing, the layer being diffusely colored. Neutral dyestuffs insoluble or difficultly soluble in water pass partially into the diffusely coloring soluble form 25 in a weak acid or also alkaline solution. Very suitable, for example, are those water-insoluble or difficultly soluble dyestuffs such as employed for dyeing acetate silk.

It is also possible to employ vat dyestuffs in 30 coarsely dispersed form, and to treat these with an alkaline hydrosulphite solution in the layer, whereby the layer is diffusely colored.

The diffuse coloring of the layer may be easily 35 regulated by the duration of the bath or by suitable interruption baths, such as water or like means, which act in chemical opposition to the dissolving agents, so that in case of requirement a bleeding of the dyestuff or passage of the dyestuff from one layer into the other may be prevented.

The most suitable for this purpose are solutions of precipitating agents, which are capable of causing the process of diffusion to be stopped when a sufficient diffuse coloring of the material 45 has been attained. It has been found to be of particular advantage to employ those precipitating agents, which not only prevent the diffusion but also improve the fastness or insolubility of the dyestuff, for example metal salts, such as aluminum or copper salts, which form mordants 55 or lakes, or for basic dyestuffs solutions of phosphotungstic or phosphomolybdic acid.

There is employed with advantage upon the conversion of the coarsely dispersed dyestuff, which colors the layer only very little or not at 60 all, into the coloring form one of the baths usual in photographic processes, the alkaline, acid or solvent concentration of which is adjusted according to the dyestuff employed. For example, the conversion of a dispersed dyestuff, which reacts in an alkaline agent, into the coloring form 65 may take place in the developer. If an acid medium is necessary for this purpose, there will be employed either the interrupting bath following on the developer, the acid fixing bath, or 70

a dyestuff-destroying bath, for example a solution of thiocarbamide containing mineral acid.

The dyestuff may be caused to color the layer diffusely by physical action.

5 *Examples.*—1. In a layer of resin a coarsely dispersed dyestuff is caused to diffuse by lengthy heating up to the temperature of the softening point.

2. On to the surface of a layer there is dusted 10 a fusible dyestuff in powder form which, after the exposure, is caused to color the surface diffusely by fusing.

The production of the dyestuff images in the 15 layers in accordance with the invention may take place in desired fashion according to the methods usual in the photographic and color-photographic art, preferably by local destruction of the dyestuff in accordance with earlier processes of the applicant. It is possible to produce 20 with the dyestuff in the layer for example wash-out reliefs or mordant or tanned images, or also to remove the dyestuff from the tanned points by solution.

The layers containing coarsely dispersed dyestuff 25 may be sensitized with desired substances, for example with silver halide, with light-sensitive heavy metal salts, such as those of iron or mercury, with chromates, or also with organic light-sensitive substances, such as diazo compounds. The light-sensitive substances may 30 either already be added to the emulsion or introduced subsequently into the finished layer. The most important use of the layers consists, however, in the combination with silver halide in 35 one or more layers, which if desired may be differently sensitized.

The technical advantage of the invention resides in the extensive decrease or preclusion of the interfering absorption (screening effect) of 40 the layers which contain the coarsely dispersed dyestuffs. This is particularly important in the production of color photographs and cinematograph films. According to the present invention, color photographic and cinematographic exposures 45 and copies may be made in direct fashion from colored originals, whereby the layers may be well sensitized directly for the complementary color.

A preferred form of embodiment of the invention resides in the use of photographic materials 50 having layers poured one on to the other, these layers containing different dyestuffs and possessing different spectral sensitivity. In this connection, in addition to the reduced absorption of 55 the dyestuffs, the great lack of diffusion on the part of the superimposed layers offers particular advantage. In the same manner it is also possible to produce different dyestuffs and differently color-sensitized particles of emulsion, which are 60 superimposed or juxtaposed in screen-like fashion. These are produced by mixing or remulsifying the differently colored and sensitized particles of emulsion. The dyestuff, however, may also be provided in coarsely dispersed form 65 above or below the light-sensitive layer in screen-like fashion. Further, there may be produced according to the invention not only colored light-sensitive layers, but also multi-color screens or layers which are diffusely colored subsequently 70 after the exposure. The dyestuffs may also be combined with sensitizers and auxiliary filter dyestuffs. For this purpose there may be employed filter dyestuffs which are capable of being both readily washed out as well as destroyed in 75 the treatment baths.

It is also possible to combine colorless layers or layers or particles of layers which are diffusely colored or contain dyestuff-forming substances.

The coarsely dispersed dyestuffs may also be applied above or below the light-sensitive layer with or without binding agents by dusting on or, as described above, with the assistance of solvents.

The dyestuff employed may be selected either 10 to be complementary or similar to the color sensitivity of the layer or also independently thereof. It is thereby easily possible to produce master images, the color of which is complementary to the color sensitivity of the colored 15 copying layers employed.

An additional advantage of the process according to the invention occurs in those cases 20 in which the layer contains dark dyestuffs, e. g. in connection with documental or reversal papers 25 or films, which must give dark pictures. In such cases, it would be difficult to obtain a sufficient exposure if the dyestuff is present in the layer in finely dispersed form. If, however, comparatively large dyestuff particles are in the layer, 30 there are sufficient gaps for the light to penetrate. In a similar manner gelatine layers for the chromate process can be made with coarsely dispersed dyestuffs, which are transformed after 35 exposure into a finely dispersed form.

On the layers according to the invention it is also possible to produce sound records, either 40 in colors or also in black-and-white. It was surprising in this connection that the coarsely dispersed grains of dyestuff had no adverse effect on the sharpness of the sound copy. An advantage resides in the fact that the sound may be copied with the light of the normal sound-copying machines, which is comparatively weak 45 for colored layers.

What I claim as new and desire to secure by Letters Patent is:

1. The method of producing photographic dyestuff images which comprises exposing a light sensitive silver halide emulsion layer, the said 45 layer containing coarse grains of fast dyestuff coarsely dispersed in an emulsion which will transmit light rays for which the coarsely distributed dyestuff possesses absorption properties, fastly dyeing the emulsion layer at a point in 50 the process after exposure by dissolving the coarsely dispersed coarse grains of dyestuff within the layer, developing the latent silver image and destroying the dyestuff locally proportionate to the metallic silver image.

2. The method of producing photographic dyestuff images which comprises exposing a light sensitive silver halide emulsion layer containing a fast dyestuff in the form of coarse grains 55 coarsely dispersed in an emulsion which will transmit and is predominantly sensitized for light rays for which the coarsely distributed dyestuff possesses absorption properties, fastly dyeing the emulsion layer at a point in the process after exposure by dissolving the coarse grains 60 of coarsely dispersed dyestuff within the layer, developing the latent silver image and destroying the dyestuff locally proportionate to the metallic silver image.

3. The method of producing photographic dyestuff images which comprises exposing a plurality of superimposed light sensitive silver halide emulsion layers, at least one of the said layers containing a fast dyestuff in the form 65 of coarse grains coarsely dispersed in an emul- 70

sion which will transmit light rays for which the coarsely distributed dyestuff possesses absorption properties, fastly dyeing the emulsion layer at a point in the process after exposure by dissolving the coarsely dispersed dyestuff within the layer, developing the latent silver image and destroying the dyestuff locally proportionate to the metallic silver image.

4. The method of producing photographic dye-  
10 stuff images which comprises exposing a plurality of light sensitive silver halide emulsion layers, at least one of the said layers containing a fast dyestuff in the form of coarse grains coarsely dispersed in an emulsion which will transmit and  
15 is predominantly sensitized for light rays for which the coarsely distributed dyestuff possesses absorption properties, fastly dyeing the emulsion layer at a point in the process after exposure by treating it with a solvent for the  
20 coarsely dispersed dyestuff, developing the latent silver image and destroying the dyestuff locally proportionate to the metallic silver image.

5. In a process of producing photographic dye-  
25 stuff images the steps of incorporating coarsely dispersed coarse grains of fast dyestuffs in the

light sensitive emulsion prior to exposure and dissolving the grains within the layer after exposure.

6. A light sensitive photographic material comprising a silver halide emulsion layer and 5 coarsely dispersed coarse grains of fast dyestuff within the said emulsion, the layer being adapted to transmit light of the spectral range in which the dyestuff performs maximal absorption.

7. A light sensitive photographic material comprising a silver halide emulsion layer and coarsely dispersed coarse grains of fast dyestuff within the said emulsion, the layer being adapted to transmit and predominantly sensitive to light 15 of the spectral range in which the dyestuff performs maximal absorption.

8. A light sensitive photographic material comprising a plurality of silver halide emulsion layers and coarsely dispersed coarse grains of 20 fast dyestuff within at least one of the said emulsion layers, the said one layer being adapted to transmit light of the spectral range in which the dyestuff performs maximal absorption.

BELÁ GÁSPÁR. 25